

(No Model.)

R. A. DENISON.

INSULATING ELECTRIC CABLES.

No. 334,850.

Patented Jan. 26, 1886.



WITNESSES:

Charles H. Remington  
Paul D. Gay

INVENTOR:

Russell A. Denison  
by Geo. H. Remington  
Atty.

# UNITED STATES PATENT OFFICE.

RUSSEL A. DENISON, OF PROVIDENCE, RHODE ISLAND.

## INSULATING ELECTRIC CABLES.

SPECIFICATION forming part of Letters Patent No. 334,850, dated January 26, 1886.

Application filed August 12, 1885. Serial No. 174,170. (No model.)

*To all whom it may concern:*

Be it known that I, RUSSEL A. DENISON, a citizen of the United States, residing at Providence, in the county of Providence and State 5 of Rhode Island, have invented certain new and useful Improvements in Insulating Electric Cables; and I do hereby declare the following to be a full, clear, and exact description of the invention, such as will enable others skilled in the art to which it appertains to 10 make and use the same, reference being had to the accompanying drawings, and to letters or figures of reference marked thereon, which form a part of this specification.

15 This invention relates to an armor or shield for electric wires or cables; and it consists, essentially, of a sheet or strip of asbestos paper or felting, covered on one or both sides with a layer of insulating material composed 20 of crushed fossil bituminous rock, combined with Trinidad asphalt tempered with mineral oil and cowdie gum for the purpose of rendering the sheet impervious to the action of water and air. The sheet is then covered on one 25 side with a thin layer of pulverized glass and mica, suitably tempered, after which the coated sheet is pressed or molded to produce 30 therein a series of parallel corrugations.

The invention further consists of a band-cable composed of two strips or sheets of said 35 corrugated and coated asbestos paper, between which the wires are placed and hermetically sealed by means of hot asphaltic cement, when, finally, the whole is passed between 40 heated corrugated rolls for the purpose of compressing or compacting the parts, thus forming an insulated band-cable adapted to be laid under ground and used for telegraphic, telephonic, or electric-lighting purposes, all 45 as will be more fully hereinafter set forth and claimed.

The object of this invention is to provide a band-cable with a coating or armor which is less expensive, and at the same possessing 50 greater efficiency as compared with other analogous cables heretofore in use.

The invention is illustrated in the accompanying sheet of drawings, in which Figure 1 represents a cross-sectional view of the strip 55 or web of asbestos paper or felting which forms the base of the armor. Fig. 2 is a view of the same after being coated with the layers

of asphaltic material composed of crushed fossil bituminous stone and Trinidad asphalt suitably tempered with cowdie gum and mineral oil. Fig. 3 is a cross-sectional view of the coated strip, having in addition a thin layer of pulverized glass and mica,  $b'$ . Fig. 4 is an enlarged cross-sectional view of the prepared sheet or armor after being corrugated for the 60 reception of the electric conducting-wires. Fig. 5 is a reduced view of the same. Fig. 6 is a cross-sectional view of the completed cable having three wires. Fig. 7 is a plan view of the same. Fig. 8 is a cross-sectional view 65 of the cable as provided with six wires. Fig. 9 is a cross-sectional view of a metallic trough lined with insulating material, and showing a series of cables therein as provided with my improved armor, said trough being divided 70 laterally into three divisions for the purpose of carrying three systems of cables—as, for example, telegraphic, electric-lighting, and telephonic uses—the whole being adapted to be placed under ground; and Fig. 10 represents a modification of the same, wherein a 75 wooden box or trough is used in lieu of the metallic one.

The following is a more detailed description of the invention, including the manner of 80 its construction and operation:

B, again referring to the drawings, designates the corrugated armor or shield, composed of the asbestos paper or felting base  $b$ , covered with the preserving coats or layers  $b'$ , the latter consisting of crushed or fine particles of bituminous rock combined with hot Trinidad asphalt tempered with cowdie gum and mineral oil. After this coating becomes sufficiently hardened, a final layer,  $b''$ , of pulverous glass and mica is spread evenly over the upper surface of said shield, when, finally, the strip or web is passed between corrugated rolls, or other suitable process, for the purpose of forming therein the series of concavo-convex-shaped longitudinal grooves or corrugations  $c$   $c'$ , thus completing its construction, and adapting the same ready for use. The band-cable A is composed of a series of conducting-wires,  $a$ , covered both top and bottom 95 with said shields B. The wires each are placed in a groove,  $c$ , (of the armor B,) and covered with melted asphalt or other suitable cement, after which the top portion, B, of the cable is 100

placed in position over said wires, when, finally, the whole is passed between heated rolls, or other equivalent means, for the purpose of cementing all the parts firmly together, the finished cable then appearing substantially as represented in Figs. 6, 7, 8, &c. The cable is now adapted to be laid under ground or water, and used for conducting the electric current or fluid, as desired, the shield or armor thus constructed forming a comparatively perfect insulator for the inclosed wires. The cable also will last an indefinite period, it not being subject to decomposition, the elements composing the same being practically indestructible and unaffected by heat or cold.

In Fig. 9 my improved cable is represented as lying within a metallic trough, F, which is lined with non-conducting material n—such as fossil-meal and asbestos—applied in a plastic state, the whole being covered and sealed by means of the lid or cover F'.

I am aware that it is not broadly new to arrange wires in the form of a flat-band cable, wherein said wires are separated from each other by means of insulating material.

Having thus described my invention, what I do claim as new, and desire to secure by United States Letters Patent, is—

1. As an improved article of manufacture, the insulating material for electric wires, herein described, the same consisting of the asbestos felt or paper base coated or saturated with crushed bituminous rock and Trinidad asphalt tempered with cowdie gum and mineral

oil, a layer of pulverized glass and mica spread evenly over the surface, and the whole rolled or otherwise formed into webs or sheets having a series of continuous grooves or corrugations, as and for the purposes set forth.

2. The improved corrugated armor or shield B, herein described, consisting of the asbestos base b, enveloped by the asphaltic composition b', and the thin layer b<sup>2</sup> of pulverized glass and mica covering the inner or concave surface of the said shield, substantially as shown, and for the purposes set forth.

3. The flat-band cable A, herein described, consisting of a series of conducting-wires, a, arranged within the two strips or webs of corrugated insulating material B, composed of asbestos b, covered with asphaltic composition b', and powdered glass and mica b<sup>2</sup>, all combined and arranged substantially as shown and hereinbefore set forth.

4. The combination, within the two closely-cemented corrugated strips or webs of insulating armor B, composed of asbestos, asphalt, and powdered glass and mica, substantially as set forth, of the conducting-wires a, arranged in said corrugations, substantially as shown, and for the purposes hereinbefore described.

In testimony whereof I have affixed my signature in presence of two witnesses.

RUSSEL A. DENISON.

Witnesses:

GEO. H. REMINGTON,  
CHARLES HANNIGAN.